

Oct. 23, 1945.

H. J. LUTH ET AL

2,387,595

METHOD AND APPARATUS FOR DRYING LUMBER

Filed Aug. 2, 1943

Fig. 1.



Fig. 2.



Fig. 3.



INVENTORS:

Harold J. Luth  
Sydney R. Krupnick  
By: *Paul C. S. [Signature]* Atty.

## UNITED STATES PATENT OFFICE

2,387,595

METHOD AND APPARATUS FOR DRYING  
LUMBER

Harold J. Luth and Sydney R. Krupnick,  
Muskegon, Mich., assignors to The Brunswick-  
Balke-Collender Company, Chicago, Ill., a cor-  
poration of Delaware

Application August 2, 1943, Serial No. 496,994

17 Claims.

(Cl. 34—1)

This invention relates to the drying of lumber. One object of the invention is to avoid the loss of time incident to the relatively slow process of kiln drying. Another object is to prevent internal strains in the cellular structure of the wood which result in checking, honeycombing and other defects in the dried lumber. It is also an object to provide a process in which the block or billet is heated to a substantially uniform temperature throughout. More specifically, we have developed a process which produces a high frequency electrostatic field in the body of the wood for heating it and which applies suction or partial vacuum for withdrawing the vapor in the direction of the grain of the wood and not otherwise, to prevent the undesirable effects heretofore experienced with other processes.

It is common knowledge in the art of drying lumber that as the thickness of the lumber increases, resulting in large cross-sectional areas, the drying problem becomes complicated. Because of the low thermo-conductivity of wood, it is very difficult to uniformly heat through the entire mass, or if uniform heating is accomplished, it is not possible to control the radiation of heat through the mass of lumber to obtain uniform contraction of the wood cells during the drying process.

Therefore, during the conventional methods of kiln drying lumber it is necessary to start at low temperatures with a high relative humidity, for example 110-120° F. at 80-90 relative humidity. This is done to allow the moisture of the innermost parts of the block to gradually work its way out without excessively drying the outside of the lumber. If this outside portion is dried at such a rate that the moisture from the inside cannot become uniformly distributed to the outer shell, stresses are set up in the timber, resulting in checks, honeycombing, and various drying defects.

Those familiar with the lumber art recognize that in the growth of the tree there are radial lines extending from the center outwardly toward the bark and when billets are cut from the logs some of the cuts intersect these lines. The resulting billets are not uniform in structure, and as moisture leaves the billets the shrinkage is greater at right angles to the radial lines than it is parallel to the radial lines, and it is these differential shrinkages that must be carefully considered in the drying operation.

It is not unusual in drying large billets, for example billets of cross-sectional areas running

from 20-25 square inches, to spend as much as 60 days in the kiln drying operation, starting, as mentioned before, at a low temperature and a high humidity, gradually raising the temperatures and lowering the humidity until the desired moisture content is obtained. By taking samples from the kilns it is impossible to determine whether or not the drying rate on the outside of the billet is compatible with the drying on the inside, and in the event the outer shell is drying too rapidly, the stresses set up are relieved by introducing wet steam into the kiln to relieve the strains.

With the advent of the use of high frequency oscillators for the generation of heat, experiments were made in the application of this method to the drying of lumber. At first, results were disappointing. This can be laid to the fact that high frequency or heatronic heating affects the article in the field through its entire mass, and, as a result the temperature tends to build up in the center of a wood block more rapidly than on the outside edge for the same reason that in kiln drying the reverse takes place, the reason being the insulating property of the wood. When wood is dried by this method the honeycombing and strains all reverse themselves as compared to the effects of kiln drying at too great a rate.

We have discovered a means of uniformly removing moisture from large billets without setting up these strains. To do this we control the temperature in the billet while subjecting it to a high frequency field and this control is accomplished by means of a high vacuum applied to the billet. By this method the temperature of the billet is controlled by the boiling point of the sap under vacuum, and the sap is removed as rapidly as it is vaporized, such removal being carried on uniformly throughout the cross-section of the wood. The temperature does not tend to climb abruptly and can be easily controlled as the moisture content falls.

Various apparatus can be used, of course, to achieve the conditions required, but we have found that a simple and relatively inexpensive means is to enclose the billet of lumber to be dried in a snugly fitting rubber sack and then connect the end of the sack to a vacuum pump and reduce the absolute pressure down to the order of 100 millimeters of mercury or less. The degree of pressure in terms of absolute units can, of course, vary. We have obtained satisfactory results operating from 80-100 millimeters and can speed up the operation by still further lowering the absolute pressure.

With such a process there is also atmospheric pressure exerted through the flexible wall of the sack on the longitudinal surfaces of the block or billet being dried, roughly 13-14 pounds per square inch; this assists in the collapsing of the cells and also minimizes the tendency toward the development of stresses.

By way of illustration the drawing shows, somewhat diagrammatically, apparatus adapted to perform the drying process in accordance with this invention.

In the drawing:

Fig. 1 is a diagrammatic representation of such apparatus in which suction is applied only to one end of the block or billet and vapor is drawn from the billet through that end only; this arrangement includes means for condensing the vapor.

Fig. 2 is a diagram representing a similar apparatus but with provision for applying a partial vacuum to both ends of the billet simultaneously and thus drawing off the vaporized sap or moisture from both ends at the same time.

Fig. 3 is a diagram of an apparatus by which suction is applied to one end of the billet while the opposite end is left open so that air can be drawn through the billet to aid in carrying off the moisture.

While the drawing illustrates certain preferred forms of apparatus and while certain preferred methods are described herein, it is to be understood that the invention is not limited to the particular form and arrangement of apparatus herein shown or to the specific procedure disclosed, it being contemplated that various changes may be made by those skilled in the art without departing from the spirit and scope of the invention as set forth in the appended claims.

Referring to the drawing, there is indicated at 1 suitable means for supplying high frequency alternating current including an oscillator and other electrical apparatus properly connected and arranged in a circuit for this purpose in accordance with well known principles. Leading from the generator 1 there are conductors 2 and 3 extending respectively to radiating plates or electrodes 4 and 5 shown spaced apart at opposite sides of the block or billet 6 which is to be treated. The block of wood 6 is herein shown as a rough turned billet of the type from which bowling pins are made and may be understood to be a green undried billet of maple wood approximately 5 inches in diameter at the largest portion and about 18 inches in length. The billet is enclosed in a snugly fitting rubber sack 7 having walls about one-eighth of an inch thick which substantially seal the surfaces of the billet which they cover.

In the form shown in Fig. 1 the sack 7 has an end wall 7a fitting against one end of the block or billet 6, but at the other end the sack is closed by a plug 8 around which its side wall may be secured in air-tight relation as by a clamping ring 9. In this figure of the drawing we have included means employed in our initial experiments for observing and measuring the actual quantity of moisture removed from the block 6. The plug 8 has a bore 10 into which there is connected an outlet pipe 11 provided with a control valve 12 and leading to a vapor condenser comprising a chamber 13 with a cooling water coil 14 extending through it. A delivery pipe 15 leads from the condenser chamber 13 to a collector bottle or equivalent receiver 16 and a suction pipe 17 leads from the top of

the bottle 16 to a suction creating pump 18 of any suitable construction.

It will be understood that the application of partial vacuum to the porous structure of the wood billet 6 reducing the pressure therein will also lower the temperature at which the sap and other moisture in the wood will evaporate. The application of a moderate quantity of heat to the billet will therefore expedite the vaporization of liquids therein and the application of suction or partial vacuum to the end of the billet will carry off the vapor as rapidly as it is formed. To avoid applying excessive heat to the billet, means for observing the temperature is shown installed in the outlet pipe 11, comprising a thermocouple indicated at 19 connected to a potentiometer 20 for registering the temperature of the vapor issuing from the billet 6. We also prefer to include a suitable gauge 21 applied to the suction line, as by connection into the bottle 16, so that the suction created by the vacuum pump 18 may be constantly observed and controlled in accordance with the best practice determined by experience.

With the apparatus set up as shown in Fig. 1, the open end of the rubber sack 7 is tightly connected to the vacuum pump 18 with the condenser 13 disposed between the sack and the pump and with the collection bottle 16 in the line between the condenser and the pump. The two radiating plates or electrodes 4 and 5 are placed at opposite sides of the billet and slightly spaced therefrom. It has been found satisfactory to employ a one kilowatt high frequency oscillator, at 1, having an output of approximately 1300 B. t. u.'s per hour and operating on 1200 cycles.

The vacuum is started up by reducing the pressure to about 80 millimeters absolute pressure and the oscillator is placed in operation. The ambient temperature conditions at the start are approximately 80° F. At the end of 30 minutes the temperature within the block will have risen to 120° F., and the first few drops of distillate will be obtained; and at the end of 30 minutes approximately 100 cc. of liquid should be distilled and the temperature will have reached approximately 132° F. In the next 30 minutes the temperature should rise to approximately 137° F. and 200 cc. of distillate is obtained, and in the next 70 minutes the final temperature will have risen to about 148° F. and a total of 500 cc. or about 1 pound 3 ounces of moisture will be distilled off and collected at 16. It has been noted that the temperature rises of its own accord toward the end of the distillation. This can be controlled by varying the output of the oscillator and by altering the degree of vacuum applied to the block.

The economy that can be effected by this method of drying is quite obvious. By rough calculation it requires approximately 1½-2½ kilowatts to effect a complete drying and the power consumption is in proportion to the reduction in moisture. It has also been found that when the wood block is unusually wet it is not necessary to immediately apply the high frequency heating. In cases where we have taken timber fresh from the woods with moisture content as high as 65-75%, in about one hour or less we have distilled off under high vacuum enough water under ambient conditions to bring the moisture content down to about 20-22%, and it is therefore necessary only to apply heat during the secondary stage of the drying.

With the apparatus shown in Fig. 2 the mode of operation will be quite similar, but the time involved may be somewhat reduced and the process accelerated because with this arrangement the rubber sack or sheath 30 is provided with two heads 31 and 32 respectively disposed adjacent opposite ends of the billet 6 and closing opposite ends of the tubular sheath 30, and these heads are fitted with outlet pipes 33 and 34 respectively, both connected to the delivery tube 35 which leads to the vacuum pump 38. With this arrangement and with a vacuum pump of suitable capacity the vaporized liquid may be withdrawn simultaneously from both ends of the billet 6.

For commercial purposes there will be no need of actually condensing the vapor after it has been once withdrawn from the billet, and the condenser and collector bottle are therefore dispensed with. Similarly, with the apparatus shown in Fig. 1, the condenser 13 and collector 16 may be omitted in commercial practice.

It will be understood that the foregoing description illustrates the principles of the invention although the mechanical setup for performing it may be varied considerably, as by changing the shape and location of the electrodes and the particular means for applying suction to the billet 6. For example, we have been able to somewhat speed up the drying time by means of a partial vacuum and a current of air pulled in a direction parallel to the grain of the block by leaving one end of the block open and depending upon resistance to the flow of air through the billet to build up the low pressure therein. Fig. 3 shows an apparatus arranged to operate in this way. The rubber sheath 40 is open at one end, leaving the end grain of the billet exposed to the air. The other end of the sheath is provided with a head 41 from which an outlet pipe 42 leads directly to the vacuum pump 43. By this method more economy is effected in the use of comparatively dry air entering one end of the billet and picking up moisture on its way through and thus speeding up the operation. Obviously, however, this requires a greater power input into the source of vacuum in order to remove the non-condensable gases from the free air flowing through the billet, and therefore this method may not offer any substantial advantage over that already described. In practice we have preferred to operate with the sack closed to the outer atmosphere as in Figs. 1 and 2, since with this arrangement it is possible to more accurately control the operation.

We have been successful in drying billets approximately 5½" in diameter and 18" long in about 2 hours and 15 minutes. The billets originally weighed 7 pounds 4 ounces and when dried weighed about 6 pounds 1 ounce and had a final moisture content of approximately 7%. The original block contained approximately 23% moisture. The actual amount of water removed was approximately 1 pound 3 ounces. The finished billets showed perfect drying conditions free from honeycombing, case hardening, and had no evidence of checks or strains when thin sections were cut parallel to the radial lines, split apart and rematched together.

We claim:

1. The method of drying a block of wood which includes substantially sealing the entire surface thereof which extends in the general direction of the grain, internally heating the block and simultaneously extracting vapor from the block

by suction applied to an end surface of the block extending across its grain.

2. The method of drying a block of wood which includes substantially sealing the surfaces thereof which extend in the general direction of its grain, applying suction thereto in the direction of said grain, and simultaneously heating the block internally to expedite vaporization of the moisture therein.

10 3. The method of drying a block of wood which includes encasing it in a snug-fitting flexible sheath of air-tight material, applying suction to at least one end surface of the block which extends across the grain thereof, and simultaneously heating the block internally to expedite vaporization of the moisture therein.

20 4. The method of drying a block of wood as defined in claim 3, in which the internal heating is accomplished by disposing the encased block between spaced electrical conductive elements and creating a high frequency alternating potential difference between said elements.

25 5. The method of drying a block of wood which includes encasing it in a snug-fitting flexible sheath of air-tight material, and applying suction to both ends of the block simultaneously while heating the block internally by means of a high frequency electrostatic field.

30 6. The method of drying a block of wood which includes enclosing the surfaces thereof which extend substantially parallel to the grain in an air-tight encasement in contact with said surfaces, applying suction to an end surface of the block extending across the grain, and simultaneously subjecting the block to a high frequency electrostatic field.

35 7. The method of drying lumber which includes enclosing the surfaces of the lumber parallel to the grain in an air-tight encasement in contact with said surfaces, applying reduced pressure to one end of the lumber and thereby drawing air through it in the direction of the grain, and simultaneously subjecting the lumber to a high frequency electrostatic field.

45 8. The method of drying a block of wood which includes substantially sealing the surfaces thereof which extend substantially parallel to the grain in an air-tight encasement in contact with said surfaces and applying suction to an end surface of the block extending across the grain.

50 9. The method of drying a block of wood which includes sealing the entire surface thereof which extends substantially parallel to the grain and applying suction to an end surface of the block extending across the grain.

55 10. The method of drying a block of wood which includes sealing all surfaces of the block except one which extends across the grain, and applying suction to said one surface.

60 11. The method of drying a block of wood which includes sealing all the surfaces thereof which extend substantially parallel to the grain and applying suction simultaneously to opposite end surfaces extending across the grain.

65 12. The method of drying a block of wood which includes sealing all the surfaces thereof which extend substantially parallel to the grain, applying suction to an end surface of the block extending across the grain, and simultaneously admitting relatively dry air to an opposite end surface of the block.

70 13. Apparatus for drying a block or billet of wood including a sheath impervious to air fitted snugly over the surfaces of the block which extend in the general direction of its grain, means

closing the ends of said sheath, an outlet leading from one of such closing means, and suction producing means, with a conduit directly connecting the suction producing means to said outlet of the closing means.

14. Apparatus for drying a block or billet of wood including a sheath impervious to air fitted snugly over the surfaces of the block which extend in the general direction of its grain, means closing the ends of said sheath with outlets leading from said end closing means, and suction producing means, with a conduit directly connecting said suction producing means to both outlets of the closing means.

15. Apparatus for drying a block or billet of wood including a sheath impervious to air fitted snugly over the surfaces of the block which extend in the general direction of its grain, means closing one end of said sheath, an outlet leading from said closing means, and suction producing means, with a conduit directly connecting said suction producing means to said outlet of the closing means, the other end of the sheath being open, exposing to the air an end surface of the block which extends across the grain.

16. Apparatus for drying a block or billet of

wood including a sheath of flexible material impervious to air and adapted to fit snugly over the surfaces of the block which extend in the general direction of its grain, means closing the ends of said sheath, an outlet conduit leading from at least one of such closing means, suction producing means, with a conduit directly connecting said suction producing means to said outlet of the closing means, a pair of electrically conductive elements spaced from said sheath at opposite sides thereof, and a high frequency alternating current generator connected to said elements.

17. Apparatus for drying a block or billet of wood including a sheath of rubber adapted to fit snugly over the surfaces of the block which extend in the general direction of the grain, means closing the ends of said sheath, an outlet in one of such end closing means, a vacuum pump, a conduit directly connecting said pump with said outlet, a pair of electrically conductive radiating plates spaced from said sheath at opposite sides thereof, and a high frequency alternating current source connected to said plates.

25

HAROLD J. LUTH.  
SYDNEY R. KRUPNICK.